

Oct. 15, 1929.

W. L. EGY

1,731,848

LIMB FOR SURVEYING INSTRUMENTS

Filed Jan. 3, 1928

2 Sheets-Sheet 1

Fig. 1.



Fig. 2.



Fig. 3.

Inventor

Willard L. Egy.

By

Dodge & Amo.

Attorneys

Oct. 15, 1929.

W. L. EGY

1,731,848

LIMB FOR SURVEYING INSTRUMENTS

Filed Jan. 3, 1928

2 Sheets-Sheet 2

*Fig. 4.*



## UNITED STATES PATENT OFFICE

WILLARD L. EGY, OF TROY, NEW YORK, ASSIGNOR TO W. & L. E. GURLEY, OF TROY,  
NEW YORK, A CORPORATION OF NEW YORK

## LIMB FOR SURVEYING INSTRUMENTS

Application filed January 3, 1928. Serial No. 244,290.

This invention relates to geometrical instruments and resides in improvements in the graduated limbs and verniers and the like forming parts of such instruments, and particularly those used in surveying instruments.

It has long been standard practice to engrave limb and vernier graduations on sterling silver because silver is capable of receiving very fine sharp engraved lines, and is of a very desirable color for the purpose. These advantages were considered so outstanding that, prior to the present invention, silver had displaced all other metals for this purpose in fine instruments, despite the well known disadvantages residing in its use.

Silver is relatively so expensive, and has such poor mechanical strength, that it must be mounted on some other support, and is so soft that the edges of the limbs must not be handled, else the edges will become rounded, destroying the sharpness and accuracy of the readings against the verniers customarily used therewith. It tarnishes readily, and when tarnished the engraved scale is illegible, particularly in poor lights.

The present invention is based on the discovery that a known alloy heretofore used in other arts merely for its lightness and high mechanical strength, offers an ideal combination of properties for this special field of use.

It is inexpensive as compared with silver, and since it can be forged into the desired forms, the limbs can be made in one piece which directly receives the graduations.

This is advantageous from the standpoint of manufacturing, simplicity and maintained accuracy. The alloy has a good texture when polished, does not tarnish from contact with the atmosphere, and can be as finely and as readily graduated as can silver. It is so hard that it resists wear, and when properly heat-treated is peculiarly free from any tendency to warp.

The freedom from warping is a property of peculiar importance in the limbs of precision instruments. The bronze heretofore used is subject to warping, as is well known to instrument makers, and limbs formed of it often warp out of round or out of plane, or both, with harmful results. The limb should

run in plane with the vernier with the edges as close together as is mechanically possible. Slight departures from accuracy in this respect limit the precision of readings. If the limb warps out of round after graduation the graduations themselves are inaccurate.

The alloy in question is an aluminum-base alloy described and claimed in the patent to Archer and Jeffries, No. 1,472,739, dated October 30, 1923. Broadly stated, the alloy is free from copper, except as an impurity and contains magnesium and not less than 0.5% silicon; preferably about 1.0% of each of magnesium and silicon. Specific examples are given in the patent above identified. The alloy develops the desired physical properties for this use by being heated, quenched and artificially aged as described in that patent.

Prior to my invention the high tensile strength, elongation and Brinell hardness of this alloy were known; but, so far as I am aware, its unusual property of receiving very sharp engraved lines, its freedom in a truly remarkable degree from any appreciable tendency to warp, its good color and surface texture, for graduated limbs, and its resistance to tarnish had neither been observed nor appreciated.

Actual use of the alloy in commercial instruments has indicated that the alloy eventually will displace silver for this use, unless something still better be found, and that it leaves little to be desired in the way of improvement.

In practice blanks for the limbs are preferably die forged in one piece, and hence require a minimum of machine finishing, but they might be cut and shaped from forged, hammered, rolled, or other mechanically worked stock, in any known manner. The blanks are heated, quenched and artificially aged before machining, and after machining are polished over the area to be graduated. They are engraved in ordinary dividing engines in the usual manner. Unfinished areas may be lacquered if desired.

In order to show different specific forms of limbs to which the invention is peculiarly applicable, it is illustrated in the accompanying drawing as embodied in a vertical limb

and vernier and in a horizontal limb and vernier for a transit of known construction.

In the drawing,—

Fig. 1 is an elevation of the vertical limb and vernier.

Fig. 2 is a section on the line 2—2 of Fig. 1.

Fig. 3 is a fragmentary section on the line 3—3 of Fig. 1.

Fig. 4 is a plan view of the horizontal limb and verniers.

Fig. 5 is a section on the line 5—5 of Fig. 4.

Referring first to Figs. 1, 2 and 3, the vertical circle in the example illustrated consists of a wheel having a central hub 6, radial spokes 7 and rim 8. The hub is provided with a cruciform opening 9 whose shape is dependent on the mode of mounting the circle on the telescope trunnion. The vertical circle is fixed in place on the trunnion by means of screws passing through the holes 11 which are formed with countersinks for the screw heads as clearly shown. The plane face 12 of the rim is machined and polished to give a good matte texture and the edge of the rim 25 is machined square with sharp edges, as indicated at 13 to run true against the vernier indicated generally by the numeral 14.

The groove 15 is a clearance groove to permit the periphery of the graduated portion 30 of the rim to be machined to a sharp edge. The vernier 14 is of the usual arcuate form and has a thin overhanging edge 16 opposed to the periphery of the limb. The vernier is mounted on the telescope standard (not 35 shown) by screws threaded into the holes 17.

Turning now to Figs. 4 and 5, a horizontal limb with two opposed verniers are shown, with all supporting parts omitted.

The limb 21 is saucer shaped, as shown in 40 Fig. 5 and the inner edge 22, adjacent the graduations, is undercut to permit this edge 22 to be machined accurately with sharp square edges. The vernier 23 is also undercut so as to present a relatively thin and 45 squared projecting portion 24 in opposition to the inner periphery of the limb.

The limb 21 is open at its center and is formed with an annular shoulder 25 which 50 centers it on the supporting flange carried by a tapered quill shaft, not shown. The limb is attached to the flange by screws which pass through the holes 26 and these holes are formed with countersinks for the screw heads, as is clearly shown.

55 No patentable invention is here claimed involving the mode of mounting either the vernier or the limb, and consequently all such features have been omitted from the drawing.

60 After the limb, formed in either of the two ways above described, or in any other suitable way, has been machined, the face to be graduated is polished by known methods and then engine divided. No special procedure is 65 necessary in either of these operations. After

the engraving operation (performed by the dividing engine) the graduations are filled to make them more legible, as is usual in this art.

Blanks for either type of limb, or for other types known in the art, may be die forged 70 from this alloy and this practice is desirable because it produces a superior blank and one which requires a minimum of machine finishing. The blank may be formed, however, by 75 cutting operations, provided the stock from which it is formed has been mechanically worked to refine it. In any case, at some time in the process of manufacture, prior to the final machining operations, the material is 80 heat-treated, that is it is quenched from the proper temperature and then artificially aged as described in the patent above identified.

In the present specification and claims the term "mechanically worked" is used as a 85 generic term inclusive of forging, hammering and rolling operations practiced to refine and improve the homogeneity of the metal.

The resulting product has a mechanical 90 strength far in excess of cast bronze heretofore almost universally used as a support for applied silver dials. The limb is devoid of any tendency to warp and is so hard that wear on the graduated edge is negligible. The 95 color is good. The polished surface will not tarnish when exposed to air (it is affected by certain gases not ordinarily encountered, notably chlorine), can readily be graduated with lines as fine and as sharp as it is possible to produce on silver, and has the advantage of light weight.

The invention offers peculiar advantages in all graduated limbs including verniers, but is particularly advantageous in any graduated limb which is read against the vernier because the freedom from warping tendency allows the use of minute clearances and assures the maintenance of absolute trueness which not only facilitates accurate reading 100 but assures the maintained accuracy of the graduations.

What is claimed is,—

1. A graduated limb having its graduated face engraved in a mechanically worked, 115 quenched, and artificially aged aluminum-base alloy, free from copper except as an impurity and containing magnesium and not less than 0.5% silicon.

2. A graduated limb having its graduated face engraved in a mechanically worked, quenched, and artificially aged aluminum-base alloy, free from copper except as an impurity and containing about 1% magnesium and about 1% silicon.

3. A one-piece graduated limb composed of an aluminum base alloy free from copper except as an impurity and containing magnesium and not less than 0.5% silicon, forged 125 to form, quenched, artificially aged, and bear- 130

ing graduations engraved directly in a polished surface of the forging.

4. A one-piece graduated limb composed of an aluminum base alloy free from copper except as an impurity and containing about 5 1% magnesium and about 1% silicon, forged to form, quenched, artificially aged, and having graduations engraved directly in a polished surface of the forging.

10 In testimony whereof I have signed my name to this specification.

WILLARD L. EGY.

15

20

25

30

35

40

45

50

55

60

65